

1

3,711,314

**METHOD OF COATING EMPLOYING ANIONIC WAX EMULSIONS**Craig C. Campbell, Cherry Hill, N.J., assignor to  
Mobil Oil CorporationNo Drawing. Filed Nov. 17, 1970, Ser. No. 90,483  
Int. Cl. B44d 1/092

U.S. Cl. 117—56

11 Claims

**ABSTRACT OF THE DISCLOSURE**

A method for coating a surface is provided which comprises contacting surfaces with an anionic wax emulsion; and thereafter contacting the wax emulsion deposited on the surface with a cationic coupling agent comprising a salt of a complex amine polymer whereby the wax particles in the emulsion are precipitated onto the surface. Articles of manufacture having surfaces coated by the above-defined method are also provided.

**BACKGROUND OF THE INVENTION****(1) Field of the invention**

This invention relates to a method for applying a coating and, in one of its aspects, relates more particularly to an improved method for applying wax particles onto a surface. Still more particularly, in this aspect, the invention relates to an improved method for the deposition of wax particles from anionic wax emulsions onto various surfaces, including articles of manufacture, plant surfaces and other forms of vegetation.

**(2) Description of the prior art**

Prior to the present invention, in order to precipitate and deposit wax particles, contained in anionic wax emulsions, in the form of external coatings or as internal sizing agents, onto various surfaces, it has been necessary to incorporate in such formulations rosin and alum, whose function was to act as precipitating agents. In addition, the presence of rosin and alum has not resulted in a neutral system. The importance of having a neutral system for deposition of wax particles is apparent from the fact that, for example, in the manufacture of coated cellulosic materials, such as paper, a neutral system makes possible improved paper gaging properties, reduction in corrosion of machinery parts, reduction in effluent disposal problems and reduction or complete elimination of expensive optical whiteners. Hence, it is highly desirable to replace the rosin and alum components with a single substituent and which would also provide a neutral system with all of the attendant economic and practical advantages.

**SUMMARY OF THE INVENTION**

It has now been found, as more fully hereinafter discussed, that surfaces can be effectively and economically coated with wax particles, by contacting these surfaces with an anionic wax emulsion, and thereafter contacting the wax emulsion deposited on the surface with a cationic coupling agent, comprising a salt of a complex amine polymer, whereby wax particles in the emulsion are precipitated onto the surface.

The use of the cationic coupling agent, in this manner, makes possible the replacement in whole, or in part, of the heretofore employed rosin and alum as precipitating agents, thereby resulting in a neutral system and affording all of the aforementioned advantages.

The sequence of first applying the anionic wax emulsion to the desired surface, followed by application of the cationic coupling agent, represents a critical condition of the coating procedure. Thus, it has been found that if

2

the wax emulsion and coupling agent are pre-mixed and the resulting mixture applied to the desired surface, there is obtained immediate and total precipitation of wax particles, resulting in the formation of undesirable globs and uneven wax deposits. On the other hand, in following the procedure in accordance with the improved method of the present invention, an even wax precipitation and distribution over the desired surface is obtained. In this respect, in accordance with one modification of the invention, the desired surface can be initially coated with a minor amount of the coupling agent and, thereafter, following contact of the thus-treated surface with the wax emulsion, the latter is then contacted with the remaining portion of the coupling agent. Such procedure can be successfully employed for facilitating attraction of the wax emulsion to the desired surface.

In carrying out the coating procedure any conventional anionic wax emulsion may be employed, from which wax particles are capable of being precipitated, and therefore may include wide varieties of anionic wax emulsions, well-known to those skilled in the art. Insofar as the surface to be coated is concerned, the deposition of the wax coating may be applied to any surface which is either anionic or cationic in nature and therefore may comprise a wide variety of articles of manufacture, plant surfaces and other forms of vegetation, including paper pulp, cotton cloth, wet process hardboard, wood and other forms of cellulosic materials.

Of special importance in carrying out the coating procedure of the present invention is the use of a cationic coupling agent. More specifically, this agent comprises a salt of a complex amine polymer which is capable of precipitating the wax particles of the emulsion onto the desired surface. Typical examples of these salts include polyamine salts obtained by reacting a reduced polyacrylamide with a fatty acid, such as formic, acetic, propionic and higher acids. Also exemplary of these salts are those obtained by the reaction of N-alkyl trimethylene diamines containing alkyl groups having at least 14 carbon atoms, with the aforementioned fatty acids.

The quantity of coupling agent employed is, preferably, that amount required for effecting precipitation of the desired amount of wax particles from the emulsion. For most purposes, the coupling agent is effectively employed in an amount from about 0.1 to about 30% and, preferably, from about 1 to about 5%, by weight, of the weight of the wax emulsion solids.

**DESCRIPTION OF SPECIFIC EMBODIMENTS**

The following examples and comparative data will serve to illustrate the novel method of the present invention for the coating of surfaces with anionic wax emulsions and the important results realized therefrom.

**Preparation of pulp slurry**

A 3% pulp slurry was prepared by (1) adding 60 grams of bleached sulphite pulp into 2 liters of distilled water and allowing the pulp to soak for a period of about 18 hours. The pulp was then disintegrated by employing 350 counter revolutions, 8750 blade revolutions, on a commercial disintegrator. The diluted pulp was then beaten (approximately 1.0% fiber slurry by total dilution to 12 liters with tap water) for a period of 3 minutes employing a one kilogram weight. Freeness, i.e. the ability of the water to drain freely from the pulp, was then measured employing 400 ml. of slurry diluted to 1000 ml. with distilled water. The oven dried weight of freeness sample was found to be 1.96 grams.

**Mixing of additives**

222 ml. of pulp slurry was taken from the beater and placed into a 800 ml. beaker so that slow stirring (approxi-

mately 60 r.p.m.) could be maintained. The fiber solution was used as taken directly from the beater at the determined 0.9% fiber solids (i.e., 1.96 grams of net pulp in 222 ml.).

#### Wax emulsion addition

1.4 ml. of anionic wax emulsion solution<sup>1</sup> (based on wax emulsion volume) was added slowly by pipette with continuous stirring. The slurry thus contained 0.014 gram of wax solids (0.71% at 1.96 grams of net fiber weight). The solution was then stirred for a period of 6 minutes.

#### Rosin addition

2.5 ml. (2.5 ml. of a fresh 1.0% rosin solution) was slowly added by pipette with continuous stirring. The slurry thus contained 0.25 gram of rosin solids (1.3% based on 1.96 grams of net fiber weight). The solution was stirred for a period of 6.5 minutes.

#### Alum addition

0.39 ml. of a fresh 10% alum solution,



was added slowly by pipette with continuous stirring. The slurry thus contained 0.39 gram of alum (2% alum based on 1.96 grams of net fiber weight). The solution was stirred for a period of 6.5 minutes.

#### Preparation of handsheet

The above-described 222 ml. of pulp solution with additives was poured into a six inch diameter Hermann handsheet apparatus. The forming cylinder was filled to the proper volume and a handsheet was formed in accordance with TAPPI Method T205.

The single handsheet was pressed on the Hermann sheet press for one minute at 50 p.s.i. diaphragm pressure. Following pressing, the handsheet was dried for 10 minutes at 240° F., employing a photographer's dryer.

As shown in the following table, with parts expressed by weight, a series of paper handsheet tests was conducted employing 20 gram batches of commercial bleached sulphite pulp. The previously described anionic wax emulsion was employed in these tests. In Examples 5 and 6 the cationic coupling agent was prepared from a polyacrylamide reduced to the amine and reacted with acetic acid. This salt was found to be cationic in character; possessed a molecular weight above about 1 million and exhibited a pH value of 1.8 in a 1% aqueous solution.

TABLE.—PAPER HANDSHEET TEST RESULTS<sup>1</sup>

| Example | Test                                               | Sizing treatment <sup>2</sup> |                          |                         |                 |                |                                               |                        | Sheet<br>wt.,<br>grams | Cobb <sup>3</sup><br>test<br>result |  |  |
|---------|----------------------------------------------------|-------------------------------|--------------------------|-------------------------|-----------------|----------------|-----------------------------------------------|------------------------|------------------------|-------------------------------------|--|--|
|         |                                                    | Percent                       |                          |                         |                 |                |                                               |                        |                        |                                     |  |  |
|         |                                                    | Free-<br>ness                 | Original<br>slurry<br>pH | Emul-<br>sion<br>solids | Rosin<br>solids | Alum<br>solids | Cou-<br>pling<br>agent <sup>4</sup><br>solids | Final<br>slurry,<br>pH |                        |                                     |  |  |
| 1       | Anionic wax emulsion and added alum to 4.5 pH      | 22                            | 5.8                      | 1                       | -----           | .3             | -----                                         | 4.5                    | 2.16                   | 207                                 |  |  |
| 2       | Anionic wax emulsion with increased alum to 3.8 pH | 21                            | 5.8                      | 3                       | -----           | 2              | -----                                         | 3.8                    | 2.14                   | 11                                  |  |  |
| 3       | Anionic wax emulsion with rosin and alum           | 24                            | 5.8                      | .7                      | 1.3             | 2              | -----                                         | 4.2                    | 2.12                   | 10                                  |  |  |
| 4       | do                                                 | 24                            | 5.8                      | .7                      | 1.3             | 1              | -----                                         | 4.2                    | 2.11                   | 11                                  |  |  |
| 5       | Anionic wax emulsion with coupling agent           | 22                            | 5.8                      | 1                       | -----           | .2             | -----                                         | 5.6                    | 2.14                   | 13                                  |  |  |
| 6       | do                                                 | 22                            | 5.8                      | 1                       | -----           | .1             | -----                                         | 5.6                    | 2.14                   | 13                                  |  |  |

<sup>1</sup> Used bleached sulfite pulp; 0.5% beater consistency in distilled water; handsheets formed in tap water. All sheets dried at 240° F./10 min. then placed in constant humidity room for 7-10 days before Cobb tests.

<sup>2</sup> Solids calculated as a percent of oven dry fiber weight.

As will be seen from the foregoing table, the series of anionic wax emulsions of Examples 1 through 6 were evaluated for Cobb Test results. In this test a relatively high numerical rating denotes a large water pick-up

| Table:                                                                 | Wt. percent |
|------------------------------------------------------------------------|-------------|
| 125/127 A.M.P. paraffin wax                                            | 53.0        |
| Microcrystalline wax                                                   | 5.0         |
| Hydrofrol acids (C <sub>14</sub> -C <sub>22</sub> fatty organic acids) | 3.5         |
| Diethanolamine                                                         | 1.5         |
| Water                                                                  | 37.0        |

(grams per square meter). Hence, a low numerical Cobb Test rating is highly desirable.

In accordance with Example 1, alum was added to the emulsion in such amount as to cause the pH to drop to a relatively low acid level (pH 4.5). Such addition, however, produced an undesirable high Cobb Test numerical rating of 207. Increasing the amount of alum, in Example 2, in order to obtain a satisfactory Cobb Test rating of 11, resulted, however, in further raising the acid level to an undesirable pH of 3.8 and also required a relatively large amount of wax emulsion.

In Examples 3 and 4, in order to obtain satisfactory Cobb Test ratings of 10 and 11, respectively, it was necessary to employ both alum and rosin.

On the other hand, as shown by Examples 5 and 6, employing small amounts of the cationic coupling agent, and in the absence of either alum or rosin, a satisfactory Cobb Test rating of 13 was obtained in each instance.

As hereinbefore indicated, the method for coating surfaces, of the present invention, is useful for treatment of a wide variety of materials and substrates and for the manufacture of various articles in which coatings of anionic wax emulsions are required. While the invention has been described with reference to preferred procedures, compositions and components therefor, it will be understood by those skilled in the art that departures from the preferred embodiments can be effectively made and are within the scope of the invention.

#### I claim:

1. A method for coating a surface, which comprises: initially contacting said surface with a minor proportion of the amount of a polyamine salt required to precipitate wax particles from an anionic wax emulsion, obtained by reacting a reduced polyacrylamide with a fatty acid, as a coupling agent; next contacting said treated surface with an anionic wax emulsion; thereafter contacting the resulting mixture with the remaining portion of said coupling agent, whereby wax particles in said emulsion are precipitated onto said surface, and thereafter drying the coating thus deposited, the minor proportion of the polyamine salt being at least about 0.1% by weight of the wax emulsion.

2. A method in accordance with claim 1, wherein said coupling agent is employed in an amount from about 0.1 to about 30%, by weight, based on the weight of the emulsion solids.

3. A method in accordance with claim 1, wherein said coupling agent applied as a 0.04% solution.

4. A method in accordance with claim 1, wherein said surface comprises a cellulosic material.

5. A method in accordance with claim 1, wherein said surface comprises paper pulp.

6. A method in accordance with claim 1, wherein said surface comprises cotton cloth.

7. A method in accordance with claim 1, wherein said surface comprises wet process hardboard.

8. A method in accordance with claim 1, wherein said surface comprises wood.

9. A method in accordance with claim 1, wherein said surface comprises vegetation.

10. A method in accordance with claim 1, wherein said coupling agent comprises a polyamine salt obtained by the reaction of an N-alkyl trimethylene diamine, containing an alkyl group having at least 14 carbon atoms, with a fatty acid.

11. A method in accordance with claim 1 wherein said coupling agent comprises a polyamine salt obtained by reacting a reduced polyacrylamide with acetic acid and having a molecular weight above about 1 million and exhibiting a pH value of 1.8 in a 1% aqueous solution.

**References Cited**

**UNITED STATES PATENTS**

|              |         |                |       |            |
|--------------|---------|----------------|-------|------------|
| 2,694,633    | 11/1954 | Pattilloch     | ----- | 162—172 X  |
| 2,487,899    | 11/1949 | Sherman        | ----- | 162—172    |
| 5 2,468,086  | 4/1949  | Latham et al.  | ----- | 117—56     |
| 2,495,283    | 1/1950  | Wernzt         | ----- | 117—161 X  |
| 2,820,719    | 1/1958  | Trusler et al. | ----- | 117—60 X   |
| 3,563,786    | 2/1971  | Tse et al.     | ----- | 117—168 X  |
| 2,603,576    | 7/1952  | Cook et al.    | ----- | 117—62.2 X |
| 10 3,247,009 | 4/1966  | Frahey         | ----- | 117—56     |
| 2,780,554    | 2/1957  | Lerner         | ----- | 117—168 X  |

WILLIAM D. MARTIN, Primary Examiner

15 M. R. LUSIGNAN, Assistant Examiner

U.S. Cl. X.R.

117—57, 60, 62.1, 143 R, 149, 158; 162—172